

# UNITED STATES PATENT OFFICE.

JAMES F. O'BRIEN, OF CHICAGO, ILLINOIS.

## EXPLOSIVE.

1,028,950.

No Drawing.

Specification of Letters Patent. Patented June 11, 1912.

Application filed September 20, 1911. Serial No. 650,373.

To all whom it may concern:

Be it known that I, JAMES F. O'BRIEN, a citizen of the United States, residing at Chicago, in the county of Cook, State of Illinois, have invented new and useful Improvements in Explosives, of which the following is a specification.

This invention relates to an explosive having as its general basis the combination of a chlorate of an alkali metal with a carbo-hydrate and a silico-aluminous substance; and it relates particularly to the use of a carbo-hydrate of the starch group in such a combination. The advantage of a carbo-hydrate of the starch group in such a combination, as over other carbo-hydrates and especially as over sugar, is this—that the starch combination cannot be ignited while the starch is moist (as in its colloidal state 10 in combination with water); and, during the process of manufacture, the starch is kept moist until the last and final operation of drying, thus completely obviating all liability of explosion. The starch carbo-hydrates also have the greater advantage of being cheaper and more readily obtainable than sugar or similar carbo-hydrates. Starch may be made in conjunction with the making of the explosive and within a powder plant; while the making of sugar requires an extensive plant, practically prohibiting the manufacture of powder and sugar together. Basically, my new explosive consists in a combination of a chlorate 20 of an alkali metal, preferably potassium chlorate, with a carbo-hydrate of the starch group, and with a silico-aluminous substance. This last named substance may be largely inert, being practically supplied as brick dust or other calcined clay. A small amount of cyanid compound, such as ferro-cyanid of potassium may be added.

The carbo-hydrate used in the explosive may be any of those compounds having the empirical formula  $C_6H_{10}O_5$ . The form known as dextrin is more easily handled as it is readily soluble in water and is, in this state, in condition to be combined with the chlorate to form the explosive. Made into the explosive it has a slightly greater explosive effect and energy than ordinary starch, although the difference is comparatively very slight.

As before noted, the starch has several advantages over the other carbo-hydrates, notably over sugar, and its most notable ad-

vantage is that of impossibility of ignition while in the process of manufacture. In my preferred process of manufacture the carbo-hydrate is first dissolved in water 60 (which may be heated) and then mixed with the other ingredients of the explosive; the whole mixture being subsequently dried and suitably divided before being ready for shipment. The starch not only has the advantage of being non-inflammable while moist, but it has the advantage of not attracting moisture when the powder is dried and ready for shipment. Other carbo-hydrates, notably sugar, will attract moisture 70 and thereby deteriorate the explosive to some extent.

The comparatively inert finely divided material (silico-aluminous substance) which I prefer to use in my explosive is finely 75 powdered brick dust or baked clay of that general character. The starch or similar compound and the chlorate are kept in the approximate proportions one to three, regardless of the amount of inert material 80 added to the powder. A typical composition would be this: three parts of potassium chlorate, one part of starch, one part of finely powdered brick dust, and, if desired, a small amount, say one or two per 85 cent. of the total of ferro-cyanid of potassium. In this combination, regardless of the presence or absence of the cyanid compound, the silico-aluminous substance enters materially into the explosive re-action; 90 and to sufficient extent to materially increase the energy of the total mass, so that, measured in terms of cost of manufacture, the explosive with the clay substance is possessed of greater energy than the explosive lacking the same. The aluminium silicates carried by the clay react with chlorin and potassium (which is otherwise left as a residue of potassium chlorid), and this re-action augments the explosive energy. 100

Having described my invention, I claim:

1. An explosive, consisting of a chlorate of an alkali metal, a carbo-hydrate of the group  $C_6H_{10}O_5$ , and a silico-aluminous substance. 105
2. An explosive, consisting of a chlorate of an alkali metal and a carbo-hydrate of the group  $C_6H_{10}O_5$  in the approximate proportions three to one, and a silico-aluminous substance.
3. An explosive, consisting of a chlorate of an alkali metal and a carbo-hydrate of 110

of an alkali metal and a carbo-hydrate of

- the group  $C_6H_{10}O_5$  in the approximate proportions three to one, and a substance containing a silico-aluminous compound.
4. An explosive, consisting of  $KClO_3$ , a member of the group  $C_6H_{10}O_5$ , and a silico-aluminous substance.
5. An explosive, consisting of  $KClO_3$ , and a member of the group  $C_6H_{10}O_5$  in the approximate proportions three to one, and a silico-aluminous material.
- 10 6. An explosive, consisting of  $KClO_3$ , a member of the group  $C_6H_{10}O_5$  in the approximate proportions three to one, and a substance containing a silico-aluminous compound.
- 15

7. An explosive, consisting of  $KClO_3$ , a member of the group  $C_6H_{10}O_5$  in the approximate proportions three to one, and burned clay.

8. An explosive, consisting of  $KClO_3$ , a member of the group  $C_6H_{10}O_5$ , and burned clay in the approximate proportions three to one to one.

In witness that I claim the foregoing I have hereunto subscribed my name this 11th 25 day of September 1911.

JAMES F. O'BRIEN.

Witnesses:

JAS. H. BALLAGH,  
JAMES T. BARKELEW.